

## UNITED STATES PATENT OFFICE

1,999,830

## STABILIZING MOTOR FUELS

William S. Calcott, Pennsgrove, N. J., and Ira E. Lee, Wilmington, Del., assignors to E. I. du Pont de Nemours & Company, Wilmington, Del., a corporation of Delaware

No Drawing. Application May 20, 1933,  
Serial No. 672,046

8 Claims. (Cl. 44—9)

This invention relates to improvements in means for stabilizing motor fuels comprising cracked hydrocarbon spirits and, more particularly, to improved materials for use with cracked 5 gasolines which may be employed as motor fuels.

It is well known that cracked gasoline tends to deteriorate on storage with the formation of 10 gummy and resinous products. Motor benzol also contains cracked hydrocarbon spirits which tend to form gummy and resinous products. It is also well known that some petroleum oils naturally contain cracked hydrocarbon spirits formed by the heat and pressure to which the 15 petroleum oil was subjected under the earth. When such a petroleum oil is subjected to distillation and the lighter or gasoline fractions collected, such gasoline fractions contain cracked hydrocarbon spirits which tend to form gummy and resinous products.

An object of the present invention is to retard the formation of gummy substances in motor fuels comprising cracked hydrocarbon spirits normally tending to form gummy substances on 20 storage. A further object is to provide new and improved means for stabilizing motor fuels. A still further object is to provide new compositions of matter comprising motor fuels normally tending to form gum and substances which retard the formation of such gum. Other objects 25 are to advance the art. Still other objects will appear hereinafter.

These objects may be accomplished according to our invention which comprises treating a motor fuel, containing cracked hydrocarbon spirits 30 normally tending to form gummy substances, with an alkoxy substituted dihydroxy benzene in an amount sufficient to retard the formation of the gummy substances. Of the alkoxy dihydroxy benzenes, we have found the methoxy dihydroxy 35 benzenes to be the most satisfactory for our purpose. The methoxy dihydroxy benzenes illustrated by phloroglucinol-mono-methyl ether have been disclosed in our Patent 1,884,559 granted October 25, 1932. Another methoxy dihydroxy benzene which we have found to be 40 particularly satisfactory is pyrogallol-1-methyl-ether.

The method employed for testing the effectiveness of the compounds used was essentially that 45 described by Voorhees and Essinger in J. S. A. E.

24, 584 (1929). In this test, 100 cc. of the cracked gasoline is heated in a glass flask under an oxygen atmosphere at 100° C. The flask is connected to a mercury manometer and the pressure observed at regular intervals. The time in 5 minutes from the start of the test until the gasoline begins to absorb oxygen, as shown by the fall in pressure, is known as the "induction period" of the gasoline. The effectiveness of a gum inhibitor is measured by the increase in induction period caused by the addition of a given 10 quantity of the inhibitor. That the induction period is directly related to gum formation can be shown by interrupting two tests of the same gasoline, one just before and the other just 15 after the induction period is reached, and determining the gum content of each sample of gasoline. The amount of gum present after the induction period is reached is several times greater than the amount present in the other sample. 20

In order to more clearly illustrate our invention and the preferred mode of carrying the same into effect, the following example is given:

## Example

25

To a gum-free unsaturated gasoline normally having an induction period of 70 minutes was added 0.004% by weight of pyrogallol-1-methyl ether. The treated gasoline had an induction 30 period of 190 minutes when subjected to the above test.

The methoxy dihydroxy benzenes may be represented by the following formula:

Pyrogallol-1-methyl ether

35



40

3-Hydroxy hydroquinone-1-methyl ether

45



50

## Phloroglucinol-mono-methyl ether



## 2-Hydroxy hydroquinone-1-methyl ether



## Methoxy-hydroquinone



25 Other mono-ethers of the trihydroxy benzenes, such as the ethoxy-dihydroxy benzenes and higher homologues may also be mentioned. However, they will be found to be less efficient on a weight basis because of their higher molecular weight.

30 The amount of the gum inhibitor which it is necessary to employ will vary with the nature and concentration of the unsaturated constituents of the cracked hydrocarbon spirits and the degree of stabilization it is desired to obtain.

35 In general, however, the concentration of the gum inhibitor in cracked gasoline will be substantially less than 0.1% by weight.

40 While we have described the preferred embodiments of our invention, it will be readily apparent to those skilled in the art that many modifications and variations may be made therein without departing from the spirit thereof. Accordingly, the scope of our invention is to be limited solely by the appended claims construed as broadly as is permissible in view of the prior art.

45 We claim:

1. Motor fuel comprising cracked hydrocarbon spirits normally tending to form gummy substances on storage having incorporated therein an alkoxy substituted dihydroxy benzene in an amount sufficient to retard the formation of the gummy substances. 5

2. Motor fuel comprising cracked hydrocarbon spirits normally tending to form gummy substances on storage having incorporated therein a methoxy substituted dihydroxy benzene in an 10 amount sufficient to retard the formation of the gummy substances.

3. Motor fuel comprising cracked hydrocarbon spirits normally tending to form gummy substances on storage having incorporated therein a 15 pyrogallol mono-alkyl ether in an amount sufficient to retard the formation of the gummy substances.

4. Motor fuel comprising cracked hydrocarbon spirits normally tending to form gummy substances on storage having incorporated therein a 20 pyrogallol mono-methyl ether in an amount sufficient to retard the formation of the gummy substances.

5. Cracked gasoline normally tending to form 25 gummy substances on storage having incorporated therein an alkoxy substituted dihydroxy benzene in an amount sufficient to retard the formation of the gummy substances.

6. Cracked gasoline normally tending to form 30 gummy substances on storage having incorporated therein a methoxy substituted dihydroxy benzene in an amount sufficient to retard the formation of the gummy substances.

7. Cracked gasoline normally tending to form 35 gummy substances on storage having incorporated therein a pyrogallol mono-alkyl ether in an amount sufficient to retard the formation of the gummy substances.

8. Cracked gasoline normally tending to form 40 gummy substances on storage having incorporated therein a pyrogallol mono-methyl ether in an amount sufficient to retard the formation of the gummy substances.

WILLIAM S. CALCOTT. 45  
IRAE LEE.